

1

3,503,087

MARKING FIBROUS MATERIAL

Hans Wolf, Wilhelm Ruettinger, and Klaus Gulbins,  
Ludwigshafen (Rhine), Germany, assignors to  
Badische Anilin- & Soda-Fabrik Aktiengesellschaft,  
Ludwigshafen (Rhine), Germany

No Drawing. Filed Apr. 5, 1965, Ser. No. 445,792  
Claims priority, application Germany, Apr. 10, 1964,

1,266,718

U.S. Cl. 8—164 Int. Cl. C09b 9/02

11 Claims 10

ABSTRACT OF THE DISCLOSURE

A process for the sighting of fibrous material with a tinting color capable of being removed therefrom by subsequent washing by applying to said fibrous material a water-soluble addition copolymer consisting essentially of an ethylenically unsaturated azo or anthraquinone dye and a water soluble comonomer.

This invention relates to a process for the temporary dyeing of fibrous material with certain water-soluble colored copolymers.

It is often necessary in the textile industry to identify fibrous material in the various phases of production by sighting colors (also called fugitive tinting colors) to avoid confusing these materials with one another. These sighting colors, with which for example fibre flock prior to spinning, the yarn or the finished cloth are identified, should remain on the fibrous material during the production phases in which they are to serve their purpose, but should be easily removable for example by washing, stripping or bleaching, at least to such an extent that they are not troublesome.

Both pigment dyes in the form of suspensions and soluble dyes of a great variety of classes, for example naphthol yellow S, azo-flavin FFN, acid violet 6BN and anthosin B, have been used hitherto depending on the type of fibrous material.

Removal of sighting colors is however usually troublesome and expensive and moreover is often incomplete; defective dyeings and diminished quality of the textiles are the consequences, especially in the case of union fabrics, because these have different affinities for the dyes.

The object of the present invention is to provide a process for dyeing fibrous material with sighting colors which are universally applicable and which can be removed again readily and without trouble in all cases.

We have found that fibrous materials of all kinds may be sighted in a very advantageous way during textile manufacture by using a water-soluble addition copolymer of:

(a) A dye having a polymerizable group outside its chromophoric system;

(b) A water-soluble comonomer containing in the molecule at least once the grouping



and, optionally,

(c) Water-insoluble comonomers.

Addition copolymers of the said type (called herein-after copolymers) and their production are known in principle. Water-solubility in this specification means the

2

property of forming with water a true or colloidal solution.

The following are examples of suitable dyes (a):



## Example 1

A rayon staple cloth is padded on a padding machine with an aqueous liquor containing 15 g./l. of a copolymer of

5 77% of acrylamide

20% of acrylic acid and

3% of the azo dye having the formula:



Examples of comonomers (b) are  $\alpha,\beta$ -unsaturated carboxylic acids having from three to six carbon atoms, such as acrylic acid, methacrylic acid, maleic acid, fumaric acid and their alkali metal salts, ammonium salts and amides, N-vinyl lactams, such as N-vinyl pyrrolidone, and 2-aminoethyl acrylate and its salts.

Examples of comonomers (c) are esters of acrylic, methacrylic, maleic and fumaric acids having one to six carbon atoms in the ester groups, acrylonitrile, vinyl esters having one to eight carbon atoms, vinyl chloride, vinylidene chloride, styrene, butadiene, ethylene and propylene, but their proportion in the copolymers should not be such as to make them insoluble in water.

The amounts of the comonomers (a), (b) and (c) may be varied within wide limits; as a rule they are from 1 to 15% for (a), from 10 to 99% for (b) and from 0 to 89% for (c), percentages in each case being by weight with reference to the total amount of the comonomers. Methods for the production of water-soluble colored copolymers are generally known so that further details need not be given.

The term colored copolymers includes copolymers in which the dye is a compound which is absorbent or fluorescent exclusively or mainly in ultraviolet light. Sighting colorations obtained with such copolymers have importance for special purposes, for example for the requirements of an automatically controlled course of manufacture.

The water-soluble copolymers to be used according to this invention have practically no affinity for the fibrous materials and also do not penetrate far into them, so that they can be removed again by simple measures, such as washing in acid, neutral or alkaline liquors. This fact, and the fact that the sighting of all kinds of fibrous from cotton to glass fibers can be effected with these copolymers in spite of their low affinity, constitute a considerable advantage over the use of conventional sighting colors. A further advantage resulting therefrom is a simplification of storage because in principle only a single type of sighting color is required for all types of fiber.

Another considerable advance is to be seen in the fact that the chemical properties of the polymeric sighting colors can be extensively adapted to the special procedures to which the fibrous material is to be subjected. For example in treatment in acid liquors sighting colors having acid groups are recommended according to this invention. After the treatment, these colored copolymers may easily be washed out by alkali. The same is true in principle for treatment of the fibrous material in alkaline liquors. The good suitability of the sighting colors according to this invention must be regarded as surprising because the strong polar water-solubilizing groups of the comonomers (b) would be expected to impart a strong affinity for fibrous materials.

A further advantage which is very important in practice is that the polymeric sighting colors according to this invention can be adjusted by choice of their composition so that they are compatible with other textile assistants and do not disturb their application or action.

The invention is further illustrated by the following examples. Percentages are by weight.



which has been neutralized with caustic soda solution.

15 The cloth is thus sighted by a tinting color having an orange pastel shade which may easily be washed out.

## Example 2

A skein of a polyester yarn is sighted by dipping it in 20 an aqueous liquor which contains 7% of a copolymer having the following composition:

70% of ethyl acrylate

7% of methyl methacrylate

10% of acrylamide

7% of sodium acrylate and

6% of the anthraquinone dye having the formula:



35 The yarn thus treated is squeezed out of a padding machine and then dried. The blue violet sighting color may be washed out easily and completely by washing with a weakly alkaline hot liquor.

40 Skeins of polyamide yarn and of acetate silk yarn may be sighted blue violet in the same way.

## Example 3

45 Yarns of cotton, wool, polyester fibers, viscose rayon, acetate rayon and polyacrylonitrile fiber are impregnated on a thread impregnating machine (comprising a liquor trough, a pair of squeeze rollers, a drying tunnel and a take-up device) successively with one and the same aqueous liquor which contains per liter

50 g. of a copolymer derived from

98% of N-vinylpyrrolidone and

2% of the azo dye having the formula:



60 The yarns are dyed yellow in this way and are then heated for fifteen minutes at 120° C.

65 After this treatment, the yarns are washed and rinsed with water at 70° C., the sighting color thus being completely removed.

We claim:

1. In a process for the sighting of fibrous material with a tinting color capable of being removed therefrom by subsequent washing, the improvement which comprises: applying to said fibrous material a water-soluble addition copolymer consisting essentially of:

(a) an azo or anthraquinone dye bearing a polymerizable vinyl group outside its chromophoric system, and

(b) a water-soluble comonomer selected from the class consisting of acrylic, methacrylic, maleic and fumaric acids and their alkali metal salts, ammonium salts and amides, N-vinylpyrrolidone, and 2-aminoethyl acrylate and its salts; drying the thus treated fibrous material; and then subsequently removing substantially all of said copolymer from the fibrous material by washing.

2. A process as claimed in claim 1 wherein the copolymer further contains:

(c) at least one water-insoluble comonomer selected from the group consisting of esters of acrylic, methacrylic, maleic and fumaric acids with one to six carbon atoms in the ester group, acrylonitrile, vinyl esters of one to eight carbon atoms, vinyl chloride, vinylidene chloride, styrene, butadiene, ethylene and propylene, in an amount such that said copolymer remains water-soluble.

3. A process as claimed in claim 1 wherein the comonomer (b) is an  $\alpha,\beta$ -unsaturated carboxylic acid selected from the group consisting of acrylic acid, methacrylic acid, maleic acid and fumaric acid.

4. A process as claimed in claim 1 wherein the comonomer (b) is an alkali metal salt of an  $\alpha,\beta$ -unsaturated carboxylic acid selected from the group consisting of acrylic acid, methacrylic acid, maleic acid and fumaric acid.

5. A process as claimed in claim 1 wherein the comonomer (b) is an ammonium salt of an  $\alpha,\beta$ -unsaturated carboxylic acid selected from the group consisting of acrylic acid, methacrylic acid, maleic acid and fumaric acid.

6. A process as claimed in claim 1 wherein the comonomer (b) is an amide of an  $\alpha,\beta$ -unsaturated carboxylic acid, selected from the group consisting of acrylic acid, methacrylic acid, maleic acid and fumaric acid.

10  
15

5

7. A process as claimed in claim 1 wherein the colored comonomer (a) is an azo dye.

8. A process as claimed in claim 1 wherein the colored comonomer (a) is an anthraquinone dye.

9. A process as claimed in claim 1 wherein the comonomer (b) is N-vinylpyrrolidone.

10. A process as claimed in claim 1 wherein the amount of comonomer (a) is from 1 to 15% by weight with reference to the total amount of comonomers (a) and (b).

11. A process as claimed in claim 2 wherein the amount of comonomer (a) is from 1 to 15% by weight, the amount of comonomer (b) is from 10 to 99% by weight and the amount of comonomer (c) is from 0 to 89% by weight with reference to the total amount of comonomers.

#### References Cited

##### UNITED STATES PATENTS

|           |        |                            |
|-----------|--------|----------------------------|
| 1,500,844 | 7/1924 | Plauson.                   |
| 2,093,651 | 9/1937 | Widmer et al. ----- 8—74 X |
| 2,473,403 | 6/1949 | Woodward ----- 8—18 X      |
| 3,190,850 | 6/1965 | Burke.                     |
| 3,232,692 | 2/1966 | Wilhelm et al. ----- 8—18  |

##### FOREIGN PATENTS

|           |         |          |
|-----------|---------|----------|
| 1,139,092 | 11/1962 | Germany. |
| 1,139,093 | 11/1962 | Germany. |

GEORGE F. LESMES, Primary Examiner

B. BETTIS, Assistant Examiner

##### U.S. CL. X.R.

8—18, 74, 177, 178, 179; 260—80.3, 80.72, 80.73

35